

May 3, 1938.

L. C. STRINGER

2,116,129

METHOD OF SEVERING AND REUNITING GLASS OBJECTS

Filed Dec. 3, 1935



INVENTOR  
L. C. STRINGER  
By C. B. Binkenbund.  
ATTORNEY.

## UNITED STATES PATENT OFFICE

2,116,129

METHOD OF SEVERING AND REUNITING  
GLASS OBJECTSLouis C. Stringer, Portland, Oreg., assignor to  
Light Service Corporation, Portland, Oreg.

Application December 3, 1935, Serial No. 52,681

## 1 Claim. (Cl. 49—77)

This invention relates generally to glass working and particularly to the method of and apparatus for severing and reuniting glass objects.

The main object of this invention is the provision of an exceedingly simple method of opening and closing a glass object and the development of suitable apparatus for use in conjunction therewith.

The second object is to make it possible to sever and reunite glass objects or to open and close glass objects such as light bulbs, radio, television, and X-ray tubes in a manner that the elements therein may be repaired, reconditioned, or rejuvenated at but a fraction of the cost of a complete replacement without distortion and resulting in a perfect union.

The third object is to make possible the improvement of the refill lamp by the utilization of those of its metallic mountings which do not require replacement and from which the oxygen has been drawn off during the previous operation of the lamp, thereby making it possible for the refill lamp to last longer than a newly manufactured one.

The fourth object is to make possible the salvaging of the more expensive portions of electrically operated appliances contained in glass envelopes by providing a completely practical method of replacing, repairing, or reconditioning the defective elements and then reenclosing it in its glass envelope.

This invention is especially applicable to devices wherein the functioning unit is contained in a vacuum and encased in a glass envelope.

These, and other objects, will become more apparent from the specification following as illustrated in the accompanying drawing, in which:

Fig. 1 is a side elevation of a representative form of tube.

Fig. 2 is an elevation similar to Fig. 1 but with a portion broken away in longitudinal section to show score marks.

Fig. 3 is a view similar to Fig. 2 showing a resistance wire disposed around the score mark.

Fig. 4 is a section taken along the line 4—4 in Fig. 3, showing the electric arrangement for the severing device.

Fig. 5 is a fragmentary section showing the severed object.

Fig. 6 is a side elevation showing a revolvable head for supporting an object while subjecting same to heat uniformly along the line where it has been severed.

Fig. 7 is a plan of Fig. 6 showing the plurality

of heating elements and their relation to the envelope.

Similar numbers of reference refer to similar parts throughout the several views.

Before entering into a description of this invention, it must be understood that it is capable of use through a very large portion of the glass working art, but is particularly well adapted to the cutting and reuniting of glass rods, tubes, lamp bulbs, or envelopes such as are used for radio, X-ray, and other appliances of a similar nature, and the explanation given herein is merely to illustrate its adaptability to the glass workers' art and the manner in which it can be used to solve the major problem in the repair of electric lamps, radio tubes, etc.

Referring in detail to the drawing, there is shown a representative form of glass envelope 10 such as is used on show case lamps which are provided with the usual base 11. It is assumed that the lamp has failed, either due to the severing of the filament or its destruction under use, and it is desired to replace the filament thereof.

If the operation to be performed is one which requires the removal of the lamp base, this is accomplished under ordinary conditions by merely heating the base 11. This may, of course, be done before or after the severing operation is performed. In order to sever the envelope or bulb

for the purpose of making the enclosed parts accessible, it is now placed in a rotating holder, not shown, where at a desired line an abrasive or scoring tool is brought into contact with the exterior of the envelope 10 while it is revolving, thereby producing the score mark 12 which encircles the envelope 10. This mark is preferably continuous but may contain one or more breaks for the purpose of producing a slight wave in the line in order to expedite the restoring of the

parts to their original relationship. It is sometimes desirable to warm the envelope 10 before it is scored. The envelope 10, after being scored, and while it is at a normal temperature, is now encircled by a resistance wire 13, which is brought into register with the score mark 12, and placed in series with a small step-down transformer 14 and the rheostat 15. The purpose of this arrangement is to make it possible to sever the tube or envelope 10 in a perfectly straight plane.

The envelope 10 having been severed is now prepared for whatever operation is necessary for its restoration to usefulness. After such repair or alteration has been made, the envelope 10 is ready to be assembled. After all the details of

5

10

15

20

25

20

25

20

30

30

35

35

40

40

45

45

50

50

55

purification have been taken care of, it is placed in a chamber, not shown, within a suitable adaptor or holder 16. The holder 16 is provided with a suitable means for rotating same while the tube or envelope 10 has its longitudinal axis in a vertical position. If this be an operation which must necessarily be performed in a vacuum, then the atmosphere must be exhausted from the chamber. After the globe or envelope 10 has been preheated to a temperature of approximately 350° F., then electric energy is applied through proper conductors to suitable electrodes, not shown, so spaced and connected as to produce a series of arcs sufficient to encompass the entire circumference of the envelope 10 along the line previously severed. It must be understood that this is being done while the envelope is rotated on the holder 16 and that sufficient heat is being applied to liquefy the two ends or portions of the envelope 10, care being taken to prevent the arcs from rendering the walls liquid over too great an area, thereby causing the portion of the member being heated to bulge, buckle, or collapse. With the proper amount of care, the possibility of loss will be reduced to a minimum.

The fusing of the glass, as stated, and the weight of the uppermost portion causes the tube parts to reunite in cylindrical form, leaving little or no indication of a joint. It is, of course, understood that after this operation is complete, the tube or envelope 10 must be properly annealed.

While I have described the fusing operation as being performed by means of an electric arc, it is desirable especially with larger and heavier globes and tubes to use controlled gas flames disposed around the rotating envelope, thereby increasing the uniformity of the heat application. It must be understood that the glass articles should be properly shielded against drafts of air and shocks in order to obtain the best possible results.

By a "controlled gas flame" is meant a flame

with a knife-like edge which can be so oriented that the maximum heat will be applied to the line of contact between the two tube ends being united, it being a matter of common knowledge that the ability of even expert glass blowers to unite thin walled glass tubes with the aid of cross-fire burners is limited to tubes of relatively small diameter; but by the use of the controlled gas flame, tubes may be joined successfully and smoothly even when the tube diameter is relatively great and the wall is relatively thin. Inasmuch as this invention is particularly directed to the rebuilding of light bulbs and similar contrivances, the necks of which are fairly large in diameter and the walls of which are very thin, the use of a controlled application of heat is of utmost importance.

While reference has been made to electric lamps and the repair thereof, it must be understood that this invention relates particularly to the separation of and the reuniting of the walls of a glass envelope. While those having a circular cross section are most common, other shapes may be cut and reunited with equal success by merely providing a means for the uniform application of heat about the periphery thereof.

I am, of course, aware that in the past objects made of glass have been severed and re-united, and it is therefore not my intention to broadly cover such processes or apparatus for performing same; but I do intend to cover all such forms and modifications of my invention as fall fairly within the appended claim.

I claim:

A method of severing glass objects consisting of progressively scoring a mark along the line of severance, then applying heat along the score line with a rising temperature, the application of said heat being limited to substantially the width of the scoring and simultaneously along the length of the score mark.

LOUIS C. STRINGER.